

## UNITED STATES PATENT OFFICE

2,553,865

## CASE HARDENING COMPOSITION

Isaac Laird Newell, Wethersfield, Conn.

No Drawing. Application March 11, 1950,  
Serial No. 149,203

11 Claims. (Cl. 148—30)

1

This invention relates to a fusible salt bath for the treatment of iron or steel or ferrous alloys by a process generally known as carburizing, cementation or case hardening. More particularly the invention relates to a novel composition and method for a case hardening treatment.

Case hardening baths have long been known and used to give a surface hardness to iron and steel parts by the introduction of carbon and nitrogen into the surface of the metal. Such baths are usually composed of a cyanogen compound with or without an activating material to accelerate or control the rate of case hardening. There is also generally present such diluents as chlorides and carbonates. Cementation with carbon and nitrogen will occur slowly when mixtures of sodium and potassium cyanides are used. By the addition of such activators as the alkaline earth metals especially calcium and barium in the form of chlorides and carbonates the rate of cementation is markedly increased and a higher proportion of carbon is introduced into the metal.

There are objectionable features to each of these well known baths. For example, where the case hardening compound consists essentially of the sodium salts of cyanide, cyanate, chloride and carbonate the bath is unstable and requires frequent and large additions of cyanides. This bath is unreliable and does not give uniform depths of case.

Calcium compounds such as calcium oxide and calcium chloride are frequently used as energizers or activators for cyanide baths, and while controlled cementation is accomplished, the bath is hygroscopic and corrosive to the work and furnace parts. The work is often coated with lime salts and acid treatment is required to clean the work.

Barium compounds are also successfully used to regulate the carburizing action of salt baths but are characterized by the great difficulty encountered in cleaning the work after cementation. As with the calcium salts, the compounds of barium are difficultly soluble in water, and alkali cleaners and acid treatment is frequently necessary to clean the metal parts.

Other energizers such as fluorides are also used, but their effect is slight and results are often erratic.

I have found that a cyanide containing salt bath composition can be activated or energized by the addition of an alkali metal fluosilicate also known as silico fluoride. The resulting bath is not open to the objections cited, and in addition has the following advantages: it is completely water soluble, and treated parts when quenched in water have a clean bright finish. The carburizing action is rapid and case depths are obtained which are equivalent to those found when using barium and strontium activated baths.

2

The baths containing fluosilicates are very stable and little or no fuming or foaming is noted at operating temperatures. An added advantage is the low cost of the accelerator especially when compared to strontium and barium compounds.

The amount of fluosilicate salt necessary to produce effective activation of a carburizing bath is low, and as small an amount as 2% is sufficient in some cases. Satisfactory energizing is also obtained when as much as 20% is used, but the bath becomes somewhat viscous and tends to sludge when as much as this is used. The preferred compositions contain from 4 to 12% of the fluosilicate salt.

The following examples will serve to further illustrate the invention:

## Example 1

Iron wire having a diameter of 0.125 inch and a carbon content 0.10 percent was treated at 1600° F. in a fused salt bath of the following composition:

|                     | Parts by weight |
|---------------------|-----------------|
| Sodium cyanide      | 20              |
| Sodium chloride     | 44              |
| Sodium carbonate    | 34              |
| Sodium fluosilicate | 2               |

After an immersion time of one hour the depth of case was .012 inch and the surface was bright and file hard. The salt bath gave no evidence of sludge formation and fuming was slight.

## Example 2

A steel rod having a carbon content of 0.012 percent was immersed in a fused salt bath of the following composition:

|                        | Parts by weight |
|------------------------|-----------------|
| Sodium cyanide         | 20              |
| Sodium chloride        | 43              |
| Sodium carbonate       | 30.99           |
| Potassium fluosilicate | 6               |
| Carbon                 | .01             |

After an immersion time of one hour during which period the temperature of the bath was maintained at 1650° F., the depth of case was found to be 0.014 inch. The surface was bright and clean and file hard. No sludging, frothing or foaming was noted.

## Example 3

A case hardening bath was prepared by blending together the following materials in powder form:

|                     | Parts by weight |
|---------------------|-----------------|
| Sodium cyanide      | 20              |
| Sodium chloride     | 39              |
| Sodium carbonate    | 32              |
| Sodium fluosilicate | 8               |
| Carbon              | 1               |

The mixture was fused and maintained at a temperature of 1600° F. In order to maintain the bath level from loss due to dragout on the work and maintain activity which might have been lessened due to surface decomposition, a replenisher was added regularly at the rate of 10 percent by weight of the bath per 8 hour day, the replenisher having the following proportions:

| Parts by weight     |    |
|---------------------|----|
| Sodium cyanide      | 40 |
| Sodium chloride     | 39 |
| Sodium carbonate    | 12 |
| Sodium fluosilicate | 8  |
| Carbon              | 1  |
|                     | 10 |

Steel rods, carbon 0.20%, manganese 0.40%, phosphorus 0.04%, sulfur 0.04%, were treated in this bath and cyanide and case depths determinations made.

| Days in Operation | Cyanide Concentration in Bath (Percent Sodium Cyanide) |
|-------------------|--------------------------------------------------------|
| 5                 | 20.6                                                   |
| 6                 | 19.4                                                   |
| 7                 | 20.6                                                   |

Microscopic examinations for case depths showed the following average figures:

|        | Depth of case<br>Inches |
|--------|-------------------------|
| 1/2 hr | .010                    |
| 1 hr   | .015                    |
| 2 hrs  | .022                    |
| 3 hrs  | .027                    |
| 4 hrs  | .030                    |

#### Example 4

A steel bolt having a carbon content of 0.15 percent was treated in a fused salt bath of the following composition:

| Parts by weight      |    |
|----------------------|----|
| Sodium cyanide       | 40 |
| Sodium cyanate       | 2  |
| Sodium chloride      | 30 |
| Sodium carbonate     | 9  |
| Potassium chloride   | 5  |
| Lithium fluosilicate | 12 |
| Carbon               | 2  |

The temperature was maintained at 1700° F. and after 1/2 hr. immersion the case depth was found to be 0.011 inch.

#### Example 5

A salt bath of the following composition was fused and maintained at a temperature of 1550° F.:

| Parts by weight     |      |
|---------------------|------|
| Sodium cyanide      | 10   |
| Sodium cyanate      | 5    |
| Sodium carbonate    | 25   |
| Sodium chloride     | 34.5 |
| Sodium fluosilicate | 20   |
| Carbon              | 0.5  |

The level of the bath in the pot was maintained by the regular addition of the following mixture,

making the addition at the rate of 1/2 percent per hour.

| Parts by weight |                     |
|-----------------|---------------------|
| 5               | Sodium cyanide      |
|                 | 75                  |
| 5               | Sodium cyanate      |
|                 | 4                   |
| 5               | Sodium carbonate    |
|                 | .5                  |
| 15              | Sodium fluosilicate |
|                 | 15                  |
|                 | Carbon              |
|                 | 0.5                 |

Steel rods having a carbon content of 0.15 percent were immersed in this bath for 2 hours. A depth of case of 0.020 inch was produced.

The examples given are not intended to be complete. Other compounds used in carburizing type salt baths such as sodium fluoride, silicon carbide, silica, sodium silicate and sodium borate do not interfere with the activating action of the fluosilicate.

In practice the cyanide percentage of the bath should be determined regularly and sufficient replenisher added to keep the bath operating at a predetermined cyanide concentration. The ranges of composition of the starting salt and replenisher may be as follows:

| 30                        | Starting Salt   | Replenisher     |
|---------------------------|-----------------|-----------------|
|                           | Parts by weight | Parts by weight |
| Sodium Cyanide            | 70-40           | 40-75           |
| Sodium Cyanate            | 0-5             | 0-5             |
| Sodium Chloride           | 5-45            | 5-40            |
| Sodium Carbonate          | 5-35            | 5-20            |
| Potassium Chloride        | 0-30            | 0-30            |
| Alkali Metal Fluosilicate | 2-20            | 2-20            |
| Carbon                    | 0-2             | 0-2             |

The higher the operating temperature, the faster the rate of cementation. Temperatures as high as 1900° F. have been used without excessive frothing or foaming of the bath. And temperatures as low as 1400° F. have been employed with effective carburizing.

What is claimed is:

1. A composition of matter for a case hardening bath for iron, steel, and ferrous alloys consisting of a mixture of the following ingredients:

| 50 | Parts by weight           |
|----|---------------------------|
|    | Sodium cyanide            |
|    | 10 to 40                  |
|    | Sodium chloride           |
|    | 5 to 45                   |
|    | Sodium carbonate          |
|    | 5 to 35                   |
|    | Alkali metal fluosilicate |
|    | 2 to 20                   |

2. A composition of matter for a case hardening bath for iron, steel, and ferrous alloys consisting of a mixture of the following ingredients:

| 60 | Parts by weight           |
|----|---------------------------|
|    | Sodium cyanide            |
|    | 10 to 40                  |
|    | Sodium cyanate            |
|    | less than 5               |
|    | Sodium chloride           |
|    | 5 to 45                   |
|    | Sodium carbonate          |
|    | 5 to 35                   |
|    | Alkali metal fluosilicate |
|    | 2 to 20                   |

3. A composition of matter for a case hardening bath for iron, steel, and ferrous alloys consisting of a mixture of the following ingredients:

| 70 | Parts by weight           |
|----|---------------------------|
|    | Sodium cyanide            |
|    | 10 to 40                  |
|    | Sodium cyanate            |
|    | less than 5               |
|    | Sodium chloride           |
|    | 5 to 45                   |
|    | Sodium carbonate          |
|    | 5 to 35                   |
|    | Potassium chloride        |
|    | less than 30              |
|    | Alkali metal fluosilicate |
|    | 2 to 20                   |

4. A composition of matter for a case hardening bath for iron, steel, and ferrous alloys consisting of a mixture of the following ingredients:

| Parts by weight           |              |
|---------------------------|--------------|
| Sodium cyanide            | 10 to 40     |
| Sodium chloride           | 5 to 45      |
| Sodium carbonate          | 5 to 35      |
| Potassium chloride        | less than 30 |
| Alkali metal fluosilicate | 2 to 20      |

5. A composition of matter for a case hardening bath for iron, steel, and ferrous alloys consisting of a mixture of the following ingredients:

| Parts by weight           |              |
|---------------------------|--------------|
| Sodium cyanide            | 10 to 40     |
| Sodium chloride           | 5 to 45      |
| Sodium carbonate          | 5 to 35      |
| Potassium chloride        | less than 30 |
| Carbon                    | less than 2  |
| Alkali metal fluosilicate | 2 to 20      |

6. A composition of matter for a case hardening bath for iron, steel, and ferrous alloys consisting of a mixture of the following ingredients:

| Parts by weight           |             |
|---------------------------|-------------|
| Sodium cyanide            | 10 to 40    |
| Sodium cyanate            | less than 5 |
| Sodium chloride           | 5 to 45     |
| Sodium carbonate          | 5 to 35     |
| Carbon                    | less than 2 |
| Alkali metal fluosilicate | 2 to 20     |

7. A composition of matter for a case hardening bath for iron, steel, and ferrous alloys consisting of a mixture of the following ingredients:

| Parts by weight           |             |
|---------------------------|-------------|
| Sodium cyanide            | 10 to 40    |
| Sodium chloride           | 5 to 45     |
| Sodium carbonate          | 5 to 35     |
| Carbon                    | less than 2 |
| Alkali metal fluosilicate | 2 to 20     |

8. A composition of matter for a case hardening bath for iron, steel, and ferrous alloys consisting of a mixture of the following ingredients:

| Parts by weight     |             |
|---------------------|-------------|
| Sodium cyanide      | 10 to 40    |
| Sodium cyanate      | less than 5 |
| Sodium chloride     | 5 to 45     |
| Sodium carbonate    | 5 to 35     |
| Carbon              | less than 2 |
| Sodium fluosilicate | 2 to 20     |

9. A composition of matter for a case hardening bath for iron, steel, and ferrous alloys consisting of a mixture of the following ingredients:

| Parts by weight           |             |
|---------------------------|-------------|
| 5 Sodium cyanide          | 10 to 40    |
| Sodium cyanate            | less than 5 |
| Sodium chloride           | 5 to 45     |
| Sodium carbonate          | 5 to 35     |
| Carbon                    | less than 2 |
| 10 Potassium fluosilicate | 2 to 20     |

10. A composition of matter for a case hardening bath for iron, steel, and ferrous alloys consisting of a mixture of the following ingredients:

| Parts by weight      |             |
|----------------------|-------------|
| Sodium cyanide       | 10 to 40    |
| Sodium cyanate       | less than 5 |
| Sodium chloride      | 5 to 45     |
| Sodium carbonate     | 5 to 35     |
| Carbon               | less than 2 |
| Lithium fluosilicate | 2 to 20     |

11. A composition of matter for a case hardening bath for iron, steel, and ferrous alloys consisting of a mixture of the following ingredients:

| Parts by weight           |              |
|---------------------------|--------------|
| Sodium cyanide            | 10 to 40     |
| Sodium cyanate            | Less than 5  |
| Sodium chloride           | 5 to 45      |
| Sodium carbonate          | 5 to 35      |
| Potassium chloride        | Less than 30 |
| Carbon                    | Less than 2  |
| Alkali metal fluosilicate | 2 to 20      |

ISAAC LAIRD NEWELL.

#### REFERENCES CITED

The following references are of record in the file of this patent:

#### UNITED STATES PATENTS

| Number    | Name | Date         |
|-----------|------|--------------|
| 1,804,454 | Beck | May 12, 1931 |

#### OTHER REFERENCES

45 "Molten Salt Baths," page 7, published by Du Pont de Nemours & Co. Inc., 1946.